

# United States Patent

[19]

Bucher et al.

[11] 3,885,997

[45] May 27, 1975

[54] **METHOD OF PRODUCING A HOT ROLLED  
AND AGE HARDENED  
COLUMBIUM-BEARING STEEL PRODUCT**

[75] Inventors: **John H. Bucher; Daniel F. Jancula,**  
both of Pittsburgh, Pa.

[73] Assignee: **Jones & Laughlin Steel Corporation,**  
Pittsburgh, Pa.

[22] Filed: **June 13, 1974**

[21] Appl. No.: **479,007**

[52] U.S. Cl. .... **148/12.3**

[51] Int. Cl. .... **C21d 7/14**

[58] Field of Search ..... **148/12 F, 12.3**

[56] **References Cited**

UNITED STATES PATENTS

|           |         |                        |          |
|-----------|---------|------------------------|----------|
| 3,666,570 | 5/1972  | Korchynsky et al. .... | 148/12.3 |
| 3,761,324 | 9/1973  | Elias et al. ....      | 148/36   |
| 3,765,874 | 10/1973 | Elias et al. ....      | 148/36   |

3,849,209 11/1974 Ishizaki et al. .... **148/12 F**

*Primary Examiner*—W. Stallard  
*Attorney, Agent, or Firm*—Gerald K. White; T. A. Zalenski

[57] **ABSTRACT**

A high strength low alloy steel product consisting essentially of 0.06 to 0.14 percent carbon, 0.6 to 1.5 percent manganese, 0.02 percent maximum silicon, 0.07 percent maximum phosphorous, 0.04 to 0.12 percent columbium, balance iron is produced in the hot rolled and aged condition by hot rolling at a finishing temperature of 1550° to 1650°F, collecting the steel at a temperature of 1000° to 1250°F and age hardening by continuous heat treatment at a temperature of 1050° to 1250°F for 0.5 to 5 minutes. The above treated product may be further subjected to galvanizing.

**6 Claims, No Drawings**

**METHOD OF PRODUCING A HOT ROLLED AND AGE HARDENED COLUMBIUM-BEARING STEEL PRODUCT**

Our invention is generally related to the production of columbium-bearing high strength low alloy steel products in the hot rolled, age hardened metallurgical state and having a minimum yield strength of 80,000 p.s.i. The process generally comprises subjecting a columbium-containing, low carbon steel to a thermo-mechanical practice which produces a fine grained, 10 hot-rolled steel product in which incomplete precipitation of columbium carbides has occurred. Yield strengths on the order of 70,000 to 80,000 p.s.i. or greater are obtained at this stage. The hot-rolled strip is thereafter continuously heat-treated in order to cause further precipitation of columbium carbides and to thus obtain a minimum yield strength of 80,000 p.s.i. Such precipitation of columbium carbides or age hardening serves to increase the yield strength by about 20 3,000 to 15,000 p.s.i. Following aging, the hot-rolled and age hardened product may be galvanized in a continuous manner.

Columbium-bearing steel products are the subject of much interest and intensive effort in the art due to their desirable combination of high strength and relatively low cost. Typical of such activity are U.S. Pat. Nos. 3,010,822, 3,102,831, 3,619,303, 3,666,570, and 3,671,334 as well as an article appearing in Metallurgical Society of Transactions of the AIME, Volume 239, April, 1967, pages 478-485.

United States Patent Numbers 3,010,822, 3,102,831 and 3,666,590 relate to the controlled thermo-mechanical processing of columbium-bearing steels but do not, however, relate to an aging or precipitation heat-treatment to enhance yield strength levels. Moreover, one following the general teachings of U.S. Pat. No. 3,619,303 would be led to believe that an age hardening heat-treatment would be ineffective upon the product produced in accordance with the above three patents because of the lack of molybdenum in the respective steel compositions. U.S. Pat. No. 3,619,303 discloses a ferrite-carbide, low alloy, constructional steel which is age hardenable. This patent teaches that columbium-bearing steels of the composition described therein will not exhibit any significant change in mechanical properties upon aging unless molybdenum is present. United States Patent Number 3,671,334 is directed to strainaged articles manufactured from nitrogenized, columbium-bearing, high-strength steels. The hot-rolled product is strainaged and aged to develop yield strengths in the vicinity of 70,000 to 90,000 p.s.i. Age hardening is due to the formation of iron carbides and nitrides. Columbium functions to increase strength primarily due to its role as a grain refining agent rather than as a precipitation hardening agent. The above mentioned AIME articles discloses solution treating and aging columbium-bearing ferritic steel.

The invention is based upon the discovery that columbium-bearing high strength steels can be age hardened to yield strength levels in excess of 80,000 p.s.i. without resort to costly alloying additions such as molybdenum through use of balanced carbon and columbium contents in combination with a controlled thermo-mechanical procedure and continuous age hardening treatment. Such procedure is advantageous in that the incompletely hardened hot rolled product can be conveniently age hardened by passage through

heat-treating equipment that is located in-line with galvanizing facilities. Hence, one may advantageously employ existing equipment to perform the dual functions of age hardening and zinc coating.

5 It is thus an object of our invention to provide a process that is capable of producing an age hardened columbium-bearing steel product having a yield strength in excess of 80,000 p.s.i. and characterized by the absence of costly alloying ingredients.

It is a further object of our invention to produce a columbium-bearing galvanized steel product in the age hardened condition and having a yield strength in excess of 80,000 p.s.i.

15 These and other objectives and advantages of our invention will be apparent to those skilled in the art from the following description of the invention.

In order to produce an incompletely hardened or aged columbium-bearing hot rolled steel product and then to subsequently age harden such product to yield strength levels greater than about 80,000 p.s.i., careful control of chemical composition, thermo-mechanical processing, and heat-treatment is required. All of the above mentioned processing limits must be controlled to fall within predetermined limits in order to achieve 20 a product having the desired mechanical properties.

25 Steel suitable for use in the invention may be manufactured by any conventional steelmaking process. Typical processes include the open hearth, basic oxygen, and electric furnace processes. Following steelmaking, molten steel is cast into conventional intermediate products such as ingots, billets, or slabs and then ultimately subjected to hot rolling into a hot rolled product such as strip.

30 Steel having the chemical composition shown in Table I is suitable for use in the practice of the invention.

TABLE I

| Element     | General Range (%) | Preferred Range (%) |
|-------------|-------------------|---------------------|
| Carbon      | .06/.14           | .08/.12             |
| Manganese   | .6/1.5            | 1.0/1.2             |
| Sulfur      | .040 max.         | .025 max.           |
| Phosphorous | .07 max.          | —                   |
| Silicon     | .02 max.          | —                   |
| Columbium   | .04/.12           | .05/.10             |

50 In addition zirconium, titanium, or rare earths may be optionally present in an amount sufficient to form globular sulfides which will not become elongated during hot-rolling. This procedure enhances bendability and formability of the final product. Sulfide shape control with zirconium or rare earth additions is taught in U.S. Pat. No. 3,666,570. Further discussion of the role 55 of zirconium and rare earths as well as titanium may be found in the article, "Control of Sulfide Shape in Low Carbon Al-Killed Steel", E. J. Licky et al, Journal of Metals, July, 1965, pages 769-775.

60 Aluminum is present in an amount sufficient to produce a killed steel product. Typical aluminum concentrations for such purpose range from a minimum of 0.02 percent.

65 Nitrogen is present in residual amounts and is not purposefully added to the steels of the invention. It will be understood by those skilled in the art that residual nitrogen content may vary with the type of steelmaking process. As an example, steel produced by the open

hearth process typically contains residual nitrogen in amounts on the order of 0.002 to 0.006 percent.

Phosphorous may be present in amounts up to 0.07 percent. Higher values should be avoided due to embrittling effects. Although some degree of minimal strengthening may occur due to the formation of iron nitrides or, in the event that zirconium is employed as a sulfide shape control agent, zirconium nitrides, the primary secondary phase strengthening mechanism involves the precipitation of columbium carbides. A major factor of the invention resides in the selection of the columbium and carbon contents of the steel. The choice of the respective contents, along with the later described thermo-mechanical processing sequence, results in the incomplete formation or precipitation of columbium carbides in the hot-rolled condition. This attainment of this metallurgical state is a prerequisite for the subsequent yield strength increase obtained through age hardening. In order to obtain incomplete columbium carbide precipitation in the hot-rolled state, a relatively high columbium content and relatively low carbon content is required. The terms "relatively high" and "relatively low" are used in the context of the general ranges taught in U.S. Pat. No. 3,666,570 which discloses a general columbium content range of 0.01 to 0.08 percent and a general carbon content range of 0.06 to 0.20 percent. For purposes of our invention columbium and carbon should be generally restricted to 0.04 to 0.12 percent and 0.06 to 0.14 percent, respectively. As may be observed, columbium is maintained at a relatively high level and carbon at a relatively low level. If one were to employ relatively high columbium and carbon levels or relatively low columbium and relatively high carbon levels, complete precipitation of columbium carbides would occur and, hence, the hot-rolled product would not be age hardenable. On the other hand, relatively low columbium and carbon contents are not capable of producing a sufficient degree of age hardening to achieve yield strength levels on the order of 80,000 p.s.i. By employing the relatively high columbium and relatively low carbon levels of the invention, an ageable hot-rolled product capable of attaining a yield strength in excess of 80,000 may be obtained. Columbium and carbon contents on the order of 0.05 to 0.10 percent and 0.08 to 0.12 percent, respectively are preferred as such relatively finer control of ingredients tends to permit a greater degree of control of columbium carbide precipitation. An additional advantage associated with lower carbon levels is that of enhanced weldability.

Manganese in amounts of from about 0.6 to 1.5 percent promotes the achievement of a basic strength level to which secondary strengthening due to columbium carbide precipitation is additive. The preferred manganese range is about 1.0 to 1.2 percent and is selected so as to be generally toward the high side of the general range in order to further ensure that yield strength values in excess of 80,000 p.s.i. are attained.

Silicon is maintained at a level of 0.02 percent maximum for purposes of optimizing zinc adherence during galvanizing.

Despite the teachings of U.S. Pat. No. 3,619,303 that molybdenum in amounts of from 0.04 to 0.50 percent is an indispensable alloying element if one wishes to age harden columbium-bearing steels, we have found that if one utilizes the described chemical composition and thermomechanical practice, significant age hardening

of the hot-rolled product may be obtained. Thus, one of the major advantages of the invention is related to the ability to achieve a yield strength increase on the order of 3,000 to 15,000 p.s.i. through an age hardening treatment. This unexpected ability obviously leads to cost reductions that are of significance in the processing of large volumes of steel. The steel of the invention contains molybdenum only in residual quantities, i.e., no intentional molybdenum additions are made to the steel. Typically such levels are no more than about 0.01 or 0.02 percent. Residual levels are a function of scrap mix and other raw material input factors and consequently may vary somewhat in given instances. Generally, however, residual molybdenum does not exceed about 0.02 percent.

Having selected a steel composition that is capable of being transformed into a hot-rolled product characterized by the incomplete formation of columbium carbides, the cast or intermediate product is then subjected to hot rolling according to prescribed finishing and collection temperature ranges. Such processing parameters are necessary in order to achieve the desired precipitation state of the invention as well as a fine grain size. Fine grain sizes, typically on the order of ASTM No. 13 to ASTM No. 15, also promote high yield strength levels.

Hot-rolling should be performed with finishing temperatures on the order of about 1550° to 1650°F. Collection of the hot-rolled steel product is accomplished by either coiling or piling. Collection temperatures on the order of from 1000° to 1250°F are suitable for purposes of the invention. At this stage of manufacture, the steel typically has a yield strength of about 70,000 to about 80,000 p.s.i. or slightly higher.

Following hot-rolling, collecting, and, optionally, pickling, the steel is subjected to a continuous age hardening treatment which serves to promote further columbium carbide formation and to increase the yield strength by about 3,000 to 15,000 p.s.i. Continuous heat treatment at a temperature of from about 1050° to 1250°F for a time of from about 0.5 to 5 minutes is sufficient to attain the desired strength increase and thereby consistently produce an 80,000 p.s.i. minimum yield strength product having acceptable ductility and toughness. The choice of times and temperatures within those described above is somewhat dependent upon line speed and product thickness.

Suitable apparatus for conducting the age hardening step is a continuous annealing furnace which commonly precedes the galvanizing step in most commercial galvanizing processes for flat rolled steel products. Normally such annealing furnaces are operated at a temperature range of 1500° to 1600°F for travel time of 0.5 to 5 minutes. Such procedure would not result in the desired age hardening for the steel of the invention. Hence, it is necessary to operate the furnace at lower than normal temperatures. It is especially advantageous to employ the annealing furnace unit of a continuous galvanizing line to the product of the invention whenever it is also desired to zinc coat the steel due to the fact that the respective treatments are in-line with each other and the aged and zinc coated product is characterized by a commercially attractive combination of strength and ductility.

An example which demonstrates a specific embodiment of the invention is as follows. A steel having a composition of 0.12 percent carbon, 0.91 percent man-

ganese, 0.052 percent phosphorous, 0.025 percent sulfur, 0.053 percent columbium, 0.10 percent zirconium, 0.03 percent molybdenum, and 0.06 percent aluminum was cast and hot-rolled into a slab using conventional practices. The slab was then hot-rolled into a 0.075 inch thick coil at a finishing temperature of 1580°F and a coiling temperature of 1220°F. The as-rolled yield strength of the hot-rolled product was 84,000 p.s.i.

Following pickling to prepare the coil surface for galvanizing, the hot-rolled coil was then processed through a conventional continuous annealing furnace to effect aging and then through a galvanizing bath to produce a galvanized product. Furnace temperature was maintained at 1170°F for the front portion of the coil, 1190°F for the middle portion of the coil, and 1150°F for the back portion of the coil. Furnace time was on the order of three minutes. A 1 1/4 oz. minimum spangle zinc coating was applied to both sides of the coil. The galvanized coil was then split into two coils, A and B, for purposes of evaluation. Coils A and B represented the front and back portions of the original coil, respectively. Coil A was tested at its front portion so as to be representative of the 1170°F temperature. Coil B was tested at both ends so as to be representative of temperatures of 1190°F and b 1150°F.

The mechanical properties shown in Table II were obtained from the two test coil portions:

TABLE II

| Coil | Furnace Temp. (°F) | Orientation  | Yield Strength (k.s.i.) | Ultimate Strength (k.s.i.) | Total Elongation (%) | Hardness (R <sub>b</sub> ) |
|------|--------------------|--------------|-------------------------|----------------------------|----------------------|----------------------------|
| A    | 1170               | Longitudinal | 87.9                    | 94.0                       | 20                   | 92                         |
|      |                    | Transverse   | 86.8                    | 94.7                       | 20                   |                            |
| B    | 1190               | Longitudinal | 91.8                    | 97.4                       | 18                   | 95                         |
|      |                    | Transverse   | 91.8                    | 97.0                       | 18                   |                            |
| B    | 1150               | Longitudinal | 84.5                    | 92.1                       | 20                   | 92                         |
|      |                    | Transverse   | 88.4                    | 95.4                       | 20                   |                            |

As may be observed from the above table, the various age hardening temperatures were sufficient to produce an increased yield strength level for a steel having the composition of and processed in accordance with the invention.

We claim:

1. A process for producing a killed high strength low alloy steel product having a yield strength in excess of about 80,000 p.s.i. in the hot rolled and age hardened condition, comprising:

a. hot rolling a steel consisting essentially of 0.06 to 0.14 percent carbon, 0.6 to 1.5 percent manganese, 0.07 percent maximum, phosphorous, 0.04 to 0.12 percent columbium, molybdenum in residual quantities, nitrogen in residual quantities, balance iron, at a finishing temperature of from 1550° to 1650°F,

5 b. collecting said hot rolled steel at a temperature of from 1000° to 1250°F; and  
c. age hardening said hot rolled steel by continuously heat treating the steel at a temperature of from 1050° to 1250°F for a time of from 0.5 to 5 minutes so as to increase the yield strength of said hot rolled steel by from about 3,000 to 15,000 p.s.i.

10 2. A process for producing a killed high strength low alloy steel product having a yield strength in excess of about 80,000 p.s.i. in the hot rolled and age hardened condition according to claim 1, wherein:

15 the steel consists essentially of 0.08 to 0.12 percent carbon, 1.0 to 1.2 percent manganese, and 0.05 to 0.10 percent columbium.

20 3. A process for producing a killed high strength low alloy steel product having a yield strength in excess of about 80,000 p.s.i. in the hot rolled and age hardened condition according to claim 1, wherein:

25 the steel consists essentially of .02% maximum molybdenum.

4. A process for producing a killed high strength low alloy steel product having a yield strength in excess of about 80,000 p.s.i. in the hot rolled and age hardened condition according to claim 1, wherein:

45 said steel further consists essentially of a sulfide inclusion shape control agent selected from the group consisting of zirconium, titanium, and rare earths in an amount sufficient to form globular sulfides in the hot rolled and age hardened condition.

5. A process for producing a killed high strength low alloy steel product having a yield strength in excess of about 80,000 p.s.i. in the hot rolled and age hardened condition according to claim 1, which further includes:

passing said hot rolled and age hardened steel product through a molten zinc bath whereby said hot rolled and age hardened steel product is coated with zinc.

6. A process for producing a killed high strength low alloy steel product having a yield strength in excess of about 80,000 p.s.i. in the hot rolled and age hardened condition according to claim 5, wherein:

55 the steel consists essentially of a maximum of 0.02 percent silicon.

\* \* \* \* \*